

## UNITED STATES PATENT OFFICE

2,021,021

MANUFACTURE AND PRODUCTION OF  
HARD METAL ALLOYS

Alan Richard Powell and Ernest Robert Box, London, England, assignors to Johnson Matthey & Company Limited, London, England, a British company

No Drawing. Application October 5, 1933, Serial No. 692,357. In Great Britain October 11, 1932

3 Claims. (Cl. 75—1)

This invention relates to the manufacture and production of hard metal alloys especially useful for tipping the points of gold nibs and the points of compass needles. The best class of nib 5 is tipped with alloys having a high content of platinum group metal as such alloys, besides being extremely hard, are absolutely unaffected by any corroding agent; there exists however, a large demand for a less costly hard alloy for use 10 in tipping the nibs used in the cheaper grades of fountain pens and it is the object of this invention to provide such an alloy.

Hard alloys consisting of a carbide, boride or silicide of metals of the tantalum and tungsten 15 groups cemented with manganese or with a metal or alloy of the iron group and prepared by sintering in hydrogen bars formed by compressing intimate mixtures of the constituents have been used for tipping the ends of high speed cutting tools 20 but such alloys cannot be broken into sufficiently small pieces for use in tipping pen nibs. If these alloys be melted down in an electric furnace the resulting product is extremely hard and very difficult to break down to small pieces and even 25 when such pieces are obtained they cannot be slit when soldered on to a gold nib.

We have now found that satisfactory hard alloys for use in tipping gold nibs comprise a mixture of at least four elements at least one being 30 selected from each of the following groups, (a) tungsten, molybdenum, (50 to 75 per cent by weight), (b) iron, cobalt, nickel (5 to 25 per cent by weight) (c) platinum, ruthenium, osmium (2 to 40 per cent by weight) (d) carbon, silicon 35 boron, (0.5 to 5 per cent by weight).

The sum of the atomic percentages of the group 40 (d) elements used should be equal to or less than the sum of the atomic percentages of the group (a) elements used, and the amount of the group (b) elements used should be at least 15 atomic 45 per cent of the amount of the group (a) elements used. The alloys obtained from melting together the members of the groups (a), (b) and (d) in these proportions are exceedingly hard and generally too brittle for use in tipping nibs hence we 50 reduce the hardness by the addition of one or more group (c) elements in an amount not exceeding 40 per cent by weight of the alloy.

Of the group (c) elements platinum tends to 55 reduce the hardness and tends to increase the toughness whereas osmium and ruthenium increase the hardness and toughness.

The elements of group (d) besides hardening the alloy have a powerful deoxidizing and de-gassing action on the molten alloys so that the 55

resulting castings are dense and quite free from porosity. In addition boron imparts to the alloys a highly desirable white colour.

The best alloys are those the proportions of the components of which are within the following ranges:—

|                                    | Per cent by weight |
|------------------------------------|--------------------|
| Platinum, ruthenium, osmium        | From 2 to 40       |
| Tungsten                           | From 50 to 70      |
| Cobalt and/or nickel               | From 5 to 25       |
| Boron and/or carbon and/or silicon | From 0.5 to 5      |

Part of the tungsten, not exceeding 10 per cent by weight, may be replaced by molybdenum but an excess of the latter metal is inadvisable because 15 it forms a readily volatile oxide at the temperatures at which the points are welded onto the gold nibs or the like.

In making the alloys the constituents may be 20 mixed together in the form of powders or small grains and the mixture melted in a suitable furnace, as for example an electric furnace of the induction, resistance or arc type. We prefer however, to add the element of group (d) in the form of an alloy with the element of group (a) 25 or (b), for example carbon may be added as tungsten carbide, boron as cobalt boride, and silicon as cobalt or tungsten silicide.

The following examples give the percentage 30 compositions of hard alloys which have proved very satisfactory, but the invention is not restricted to these examples.

## Example 1

|           | Per cent by weight                                     |
|-----------|--------------------------------------------------------|
| Ruthenium | 20                                                     |
| Tungsten  | 67                                                     |
| Cobalt    | 12 and                                                 |
| Boron     | 1                                                      |
|           | the boron being added in the form of cobalt 40 boride. |

## Example 2

|           | Per cent by weight |
|-----------|--------------------|
| Platinum  | 10                 |
| Ruthenium | 15                 |
| Tungsten  | 65                 |
| Cobalt    | 9 and              |
| Boron     | 1                  |

the boron being added in the form of cobalt 50 boride.

What we claim is:

1. A hard alloy obtained by melting a mixture of from 50 to 75% of tungsten, 0.5 to 5% of

boron, 5 to 25% of an element from the group consisting of cobalt and nickel, and 2 to 40% of an element from the group consisting of platinum, ruthenium and osmium, the proportion of boron to tungsten being not greater than 11 to 184 and the proportion of the element from the group consisting of cobalt and nickel to tungsten being at least 9 to 184.

2. A hard alloy consisting of 20 per cent by

weight of ruthenium, 67 per cent of tungsten, 12 per cent of cobalt and 1 per cent of boron.

3. A hard alloy consisting of 10 per cent by weight of platinum, 15 per cent of ruthenium, 65 per cent of tungsten, 9 per cent of cobalt and 1 per cent of boron.

ALAN RICHARD POWELL,  
ERNEST ROBERT BOX.